

# UNITED STATES PATENT OFFICE.

WILLIAM C. BEYENBERG, OF PASSAIC, NEW JERSEY.

## WATERPROOF COMPOSITION.

1,390,424.

Specification of Letters Patent. Patented Sept. 13, 1921.

No Drawing.

Application filed December 1, 1920. Serial No. 427,587.

*To all whom it may concern:*

Be it known that I, WILLIAM C. BEYENBERG, a citizen of the United States, and resident of Passaic, in the county of Passaic and 5 State of New Jersey, have invented certain new and useful Improvements in a Waterproof Composition, of which the following is a specification.

The object of my invention is the production of a waterproofing, stiffening, or reinforcing composition for impregnating textile material. When applied to such material, the textile becomes waterproof, and when dry will retain any shape or form into 15 which it might be forced.

The textile material thus impregnated and made absolutely waterproof will resist any influence of moisture, thereby preventing the form imparted to that textile material being altered by exposure to rain, dampness, etc.

My composition consists of a mixture of rubber, glue, starch, gum-arabic, rosin, and water in certain proportions. In preparing 25 the composition, I prefer to use the ingredients in about the following portions: 20% of rubber in liquid form in a solvent; 10% of glue in liquid form; 20% to 25% of starch in powdered form; 5% to 10% of an 30 equal mixture of gum-arabic and rosin, powdered; and about 40% of water. This mixture is boiled until it becomes a gelatinous paste, whereafter it is filtered so as to form a homogeneous smooth mass.

35 It is used in its paste-like form and applied after having been heated, to flexible textile material which is to be impregnated thereby, prior to receiving various desired shapes impressed into this material.

40 During the impression operation, the textile material or the matrices in which the textile material is formed, is subjected to heat which quickly evaporates all the liquid

ingredients of my mixture. Through the influence of heat, the composition becomes a 45 solid residue which causes the textile material to retain the impressed shape while it simultaneously makes it impervious to water or moisture.

My composition may be used for various 50 similar purposes; but its application is particularly advantageous in producing embossed embroidered ornaments, the subject matter of which is specified and claimed by me in a separate application. Serial No. 55 427,588, filed December 1st, 1920.

My composition is inexpensive, very efficient for the peculiar use for which it is compounded and possesses all the properties required to make a textile material 60 waterproof and retain its form into which the textile is forced.

While I have mentioned certain proportions which I prefer in making my composition, be it understood that any other proportions of the ingredients might be compounded for various purposes to which my mixture can be used.

I claim:

1. A composition for waterproofing and 70 stiffening textile material which comprises a combination of rubber, glue, starch, gum-arabic, and rosin, in about the proportions herein specified.

2. A composition of rubber, glue, starch, 75 gum-arabic, rosin, and water substantially as described.

3. A partially evaporative gelatinous composition of rubber, glue, starch, gum-arabic, 80 rosin and water for the purpose herein specified mixed in the respective proportions of 20%, 10%, 20%, 5%, 5%, and 40%.

Signed at New York in the county of New York and State of New York this 24th day of November A. D. 1920.

WILLIAM C. BEYENBERG.